

Oct. 22, 1929.

R. M. ROOKE, JR.

1,732,912

METHOD OF REMOVING DEFECTS FROM STEEL BILLETS

Filed June 2, 1928

Fig. 1.



Fig. 2.



Fig. 3.



Fig. 4.



Fig. 5.



INVENTOR  
Robert M. Cooke, Jr.  
By J. F. Brandenburg  
his ATTORNEY

## UNITED STATES PATENT OFFICE

ROBERT M. ROOKE, JR., OF JERSEY CITY, NEW JERSEY, ASSIGNOR TO AIR REDUCTION COMPANY, INCORPORATED, OF NEW YORK, N. Y., A CORPORATION OF NEW YORK

## METHOD OF REMOVING DEFECTS FROM STEEL BILLETS

Application filed June 2, 1928. Serial No. 282,291.

One of the problems in the steel industry has been the removal of defects in billets, which, if not properly removed, are perpetuated in rolling or forging as flaws in the final product.

These defects are in the nature of cracks, fissures or seams extending inward from or below the surface. In the original billets, or in the material after rolling or forging, they 10 are variously known as seams, cracks, hair cracks, hair seams, lap seams, laps, cold laps, cold shuts, and snakes, a snake being a long wavy seam often found in billets. Seam may be used as a general term.

15 The usual practice is to gouge out the seam or defect with a pneumatic hammer and chisel. This has the disadvantage of being slow, and while it may be successful, it is difficult to see whether or not the channel is made 20 to the bottom of the crack, as the chisel has a tendency to cover up the defect. Moreover, the chiseling operation being laborious, the gouge may not be made wide enough, and if 25 too narrow it will be closed in by subsequent rolling or working, with the result that the defect will not be eliminated in the final product.

According to the present invention the 30 defects are gouged out by burning the metal away in an oxygen stream scooping crosswise of the defect. In this way the gouge may be made of any width and of sufficient depth with equal ease, and the defect appears to be 35 opened up and magnified, whereas when the chisel method is used it is often difficult to determine whether all the defect has been removed.

Furthermore, the present method has a 40 great advantage in speed, thereby increasing the output and reducing the labor cost. In some mills it is costing \$14.00 to \$16.00 a ton for chipping billets, which means about 1¢ per pound on the finished product. By the present method this expense is greatly reduced.

45 In the accompanying drawings forming part hereof:

Fig. 1 is a perspective view illustrating the manner of removing a defect in a billet by means of the invention;

50 Fig. 2 is an end view of the same;

Fig. 3 is a schematic view representing a portion of an end or cross-section of a billet, showing in the middle a seam, at the left a properly made gouge which has removed a defect, and at the right a gouge which has seemingly removed a defect but is too narrow; 55

Fig. 4 is a similar view of the same illustrating the effect of rolling; and

Fig. 5 is a schematic view of a portion of a billet indicating the result that would be obtained with an ordinary oxygen cutting jet if the attempt were made to remove a defect therewith. 60

Fig. 1 illustrates a billet 2 having a seam or snake 3 in one surface. A wide, shallow 65 depression including the place where the seam was has been gouged out by an oxygen stream, aided as a practical matter by heating jets, delivered from an oxyacetylene or like torch 4. A portion of the seam has been 70 removed.

Fig. 2 illustrates the position in which the tip 5 of the torch is held, at a distance removed from, and inclined crosswise of, the seam, so that the oxygen jet acts obliquely 75 downward, and then, as its velocity fails and as it is consumed, is deflected upward again, so as to burn the metal and blow out the oxide, forming the broad curved depression 6. The tip is advanced or drawn along in this manner, parallel with the seam, until the whole region has been hollowed out, leaving a gouge coextensive with the length of the former seam. The velocity of the oxygen jet must be quite low to produce this effect and not 80 85 cut a kerf.

Fig. 5 shows what would occur if the regular cutting jet were used delivered from a torch held in the same manner, the kerf 27 not only not removing the seam but constituting another defect. 90

At the left of Fig. 3 there is shown a properly formed gouge, and at the right a gouge that is too narrow. Fig. 4 shows that, after 95 rolling, the seam 3 is still present and is becoming a concealed flaw, and that whereas the properly formed gouge is being flattened out, the narrow gouge is being closed in.

The drawing indicates the head 7 and the forward portions of the pipes 8, 9 and 10 of 100

a cutting torch, the pipe 8 serving to conduct the oxygen for combustion with the metal, the pipe 9 the oxygen for the heating jets, and the pipe 10 the acetylene or other combustible gas for the heating jets. The method can be performed with an ordinary cutting tip by throttling down the oxygen sufficiently to secure the requisite low outflow velocity from the cutting jet orifice, or the torch or tip used 10 may be specially designed to deliver a low velocity stream of suitable size.

In operating on billets or the like to remove defects by this process, the seam is entirely visible at all times while the work is 15 under way, and the operator can easily regulate the depth and width of the channel so as to remove the seam entirely and leave the billet in proper condition for rolling. The tip may be inclined slightly forward, as well as 20 laterally of the seam, the particular angle of the tip and the inclination of the side of the gouge being readily determinable by the operator taking into account the speed of cutting, the gas and oxygen pressures, and the 25 shape of the channel to be made.

While the term cutting has been used, it will be understood that the action that takes place is similar to cutting only in that there is a true combustion of the metal with the 30 oxygen. Otherwise, the process is carried out in a manner entirely different from regular cutting, wherein a high velocity jet acts without deflection, and, for the cutting of kerfs through metal, the action is confined as narrowly as possible between parallel planes.

Instead of acetylene, any other suitable combustible gas may be used for the heating jets.

I claim:

40 The herein described method of preparing defective billets or the like for rolling or forging, which comprises gouging out the surface portion of the billet containing a seam or other defect by combustion with a stream 45 of oxygen of suitable velocity directed at an inclination to the surface of the metal and crosswise with respect to the direction of displacement of the stream.

ROBERT M. ROOKE, JR.